

May 19, 1953

J. C. ROEDIGER

2,638,823

ASPHALT PAVEMENT

Filed Jan. 3, 1949



Joseph C. Roediger Inventor

B. S. W. O. T. Kilmar Attorneys

## UNITED STATES PATENT OFFICE

2,638,823

## ASPHALT PAVEMENT

Joseph Carl Roediger, Brooklyn, N. Y., assignor  
to Standard Oil Development Company, a cor-  
poration of Delaware

Application January 3, 1949, Serial No. 69,032

3 Claims. (Cl. 94—9)

1

This invention relates to improvements in asphalt pavements for application over impervious bases, such as concrete and relates particularly to asphalt pavements with surfaces that are capable of withstanding long exposure to weather before the critical hardness is reached that results in cracking.

In the application of asphalt-aggregate paving mixtures over impervious bases, such as a concrete pavement, it has been found that water collects in the layer of pavement adjacent to the impervious concrete base as it cannot drain downward through the base. Long contact of this entrapped water with the asphalt mixture gradually induces the removal or "stripping" of the asphalt from the mineral particles. This action progressively proceeds upward through the asphalt mixture until failure occurs due to cracking and crumbling of the top surface of the pavement. During this progressive upward stripping action of the water, the top of the exposed pavement remains in a satisfactory unstripped condition.

Present art shows that the stripping action of the water can be overcome by the incorporation of certain asphalt wetting agents in the asphalt prior to application. Wetting agents of this type are generally heavy metal soaps, high molecular weight organic amines or nitrogenous base materials, or combinations of amine with organic acids. Another method involves pretreatment of the mineral aggregate with these wetting agents prior to application of the normal, untreated asphalt. However, these additives increase the cost of the final asphalt pavement and it is economic to reduce the quantities used to the minimum level required to meet the average stripping action encountered in road construction. Under the severe stripping conditions encountered with an asphalt pavement over concrete, higher than normal wetting agent quantities must be used to attain satisfactory results, and the resultant added cost is frequently uneconomic.

It is also known that the rate of stripping of an asphalt coating decreases as the consistency of the asphalt is increased. For example, a 100 g./5 sec./at 77° F. 41/50 penetration grade asphalt strips less from a given coated aggregate than the same aggregate coated with an asphalt of 100 g./5 sec./at 77° F. 85/100 penetration, for the same duration of water exposure. However, the pavement laid with the 100 g./5 sec./77° F. 41/50 penetration asphalt is more prone to crack on aging than one made with the softer 100 g./5 sec./77° F. 85/100 penetration grade. Due to the

10

15

20

25

30

35

40

45

50

55

2

action of sunlight, air and moisture, the asphalt in a pavement hardens with continued exposure, which is most pronounced at the top surface of the pavement where more ready access of the elements is possible. When the weathered asphalt reaches a critical hardness, the mixture begins to crack, usually from the top surface downward.

The accompanying drawing depicts a cross-section of a road constructed in accordance with a preferred embodiment of the present invention.

The present invention, then, concerns an asphaltic pavement structure that possesses improved stripping resistance as well as good weathering quality. It may be best understood by referring to the accompanying drawing which depicts a cross-section of a road constructed in accordance with a preferred embodiment of the invention. Briefly, the structure consists of three courses—a foundation course 1, a lower asphaltic course 3 and an upper asphaltic course 6.

The foundation course 1 may be constructed of any substantially water-impervious material such as concrete. It is contemplated that this course will generally be an old concrete pavement that is in need of resurfacing. It is also contemplated that this course will be primed with one of the standard asphalt primers before any asphaltic courses are applied on it.

Immediately above the foundation course is lower asphaltic course 3 composed of particles of aggregate 4, an asphalt binder 5 and an asphalt wetting agent. The asphalt binder preferably has a penetration value of 40-60 and contains an anti-stripping asphalt wetting agent in an amount 50-100 percent greater than the amount found to be the minimum level for the aggregate being used. In addition, the asphalt binder may constitute from 4% to 12% by weight of the course.

Upper asphaltic course 6 is applied directly above lower course 3 and is composed of an asphalt binder 8 and particles of aggregate 7. The asphalt binder in this course has a penetration value in the range of 70 to 100, contains no wetting agent, and may constitute from about 9.5 to 12% by weight of the course. The softer asphalt in this course will be capable of longer exposure to the weather before the critical hardness, resulting in cracking, is reached.

In summary, this combination paving construction consists of: (1) a lower course made with a relatively hard asphalt containing more than the normal amount of asphalt wetting agent in order to attain maximum resistance to the stripping

action of water, and (2) an upper course made with a softer asphalt without wetting agent in order to attain maximum resistance to cracking in a region where the stripping action of water is negligible. An economic benefit also results since the costly asphalt wetting agent shall only be used in the region where severe stripping action results.

The thickness of the layers used may be varied extensively depending upon certain traffic conditions. Where traffic is relatively heavy, a heavier under layer is used and the thickness of the center layer may be increased. The thickness of both layers may be the same or greater in one layer than the other. Likewise the compositions are varied; for example, if a smooth top layer is desired the amount of asphalt added to the mineral aggregate is increased.

The bottom course may be a 2" layer of graded aggregate asphaltic concrete prepared with a harder asphalt (40/60 penetration) than is normally specified, and containing 2 percent by weight in the asphalt of a metallic soap wetting agent, lead naphthenate. The top course would be a conventional sheet asphalt surface course of 1".

|                                      | Bottom Course                                        | Top Course |
|--------------------------------------|------------------------------------------------------|------------|
| Thickness.....                       | 2"                                                   | 1"         |
| Sieve Size:                          | Combined Aggregate plus Filler Total Percent Passing |            |
| 3/4"                                 | 95-100                                               |            |
| 1/2"                                 | 75-90                                                |            |
| No. 4.....                           | 45-60                                                |            |
| No. 10.....                          | 35-47                                                | 100        |
| No. 40.....                          | 23-33                                                | 72         |
| No. 80.....                          | 16-24                                                | 37         |
| No. 200.....                         | 6-12                                                 | 15         |
| Asphalt:                             |                                                      |            |
| Penetration 77° F./100 g./5 sec..... | 40/50                                                | 85/100     |
| Amount <sup>1</sup> .....            | 6.0-8.0                                              | 9.5-12.0   |
| Lead Naphthenate <sup>2</sup> .....  | 2.0                                                  | None       |

<sup>1</sup> Asphalt cement in pounds per 100 pounds of aggregate.

<sup>2</sup> Wetting agent in pounds per 100 pounds of asphalt.

Conventional methods are used for the preparation of the hot mixes, and their application to the road. Various conventional combinations of high type base course mixtures and surface course mixtures can be used. Other asphalt wetting agents may be advantageously employed such as other water insoluble-oil soluble heavy metal soaps made from naphthenic, oleic, palmitic, stearic acids; or organic salts made by the combination of fatty acids with selected amines, imidazolines, etc.

This new method of application is not limited to hot mix, hot laid paving mixtures, but can also be employed to the so-called cold coated mixtures made by plant mix methods—such as the macadam aggregate, dense graded aggregate

types and such proprietary mixtures as Amesite.

The wetting agents used according to this invention are lauryl amine plus fatty acid, lead naphthenate, iron naphthenate, lead oleate, iron oleate, imidazoline, heptadecylimidazoline, heptadecylimidazoline with fatty acid, tall oil, imidazoline plus fatty acid, and a sulfonic acid salt of an adhesive selected from the group consisting of cation-active organic derivatives of ammonia containing at least one lipophilic radical directly attached to a nitrogen atom of said ammonia derivative by means of a nitrogen to carbon bond, etc.

What is claimed:

15 1. An asphalt structure consisting of a substantially water-impervious pavement foundation, a lower asphalt course consisting of a relatively hard asphalt having a 100 g./5 sec./77° F. penetration of 40-60, mineral aggregate and an asphalt wetting agent, and an upper asphalt course consisting of mineral aggregate and an asphalt having a 100 g./5 sec./77° F. penetration of 70-100.

20 2. An improved age and wear-resistant asphalt pavement structure comprising a foundation course consisting of concrete, a lower asphalt course consisting of 4-12% of asphalt having a 100 g./5 sec./77° F. penetration of 40-60, a mineral aggregate and 1-5% based on the asphalt of an asphalt wetting agent, and an upper asphalt course consisting of a mineral aggregate and 9.5-12% of an asphalt having a 100 g./5 sec./77° F. penetration of 85-100.

25 3. An improved age and wear resistant asphalt pavement structure comprising a foundation course consisting of concrete, a lower asphaltic concrete course consisting of 6 to 8% of asphalt having a 100 g./5 sec./77° F. penetration of 40 to 50, a mineral aggregate and about 2% based on the asphalt of an asphalt wetting agent and an upper sheet asphalt course consisting of a mineral aggregate and 9½ to 12% of an asphalt having a 100 g./5 sec./77° F. penetration of 85 to 100.

JOSEPH CARL ROEDIGER.

References Cited in the file of this patent

UNITED STATES PATENTS

| Number        | Name      | Date          |
|---------------|-----------|---------------|
| 50 Re. 16,799 | Burdge    | Nov. 29, 1927 |
| 1,082,722     | Alexander | Dec. 30, 1913 |
| 1,845,405     | Finley    | Feb. 16, 1932 |
| 2,332,260     | Roediger  | Oct. 19, 1943 |
| 2,339,853     | Hemmer    | Jan. 25, 1944 |
| 55 2,342,861  | Hemmer    | Feb. 29, 1944 |

FOREIGN PATENTS

| Number            | Country   | Date          |
|-------------------|-----------|---------------|
| 60 23,881 of 1935 | Australia | Dec. 10, 1936 |